

## 1

3,705,823

### METHOD OF COATING FIBROUS STRUCTURE WITH A MIXTURE OF POLYURETHANE PRE- POLYMER AND POLYORGANOSILOXANE

Kenjiro Hosokawa and Michio Ichikawa, Osaka, Japan,  
assignors to Kanegafuchi Boseki Kabushiki Kaisha,  
Tokyo, Japan  
No Drawing. Filed July 30, 1970, Ser. No. 59,721  
Claims priority, application Japan, Aug. 5, 1969,  
44/61,804

Int. Cl. D06m 15/52, 15/06; B44d 1/46  
U.S. Cl. 117—161 KP 16 Claims

#### ABSTRACT OF THE DISCLOSURE

Improved fibrous structures such as fibers, yarns, fabrics, made-up clothes and the like, having voluminous hand, durable elasticity, excellent anti-pilling property, shrink-proofness, crease resistance, and other desirable chemical and physical properties, are manufacturable by finishing the fibrous structure with a non-aqueous organic solvent solution of a specified polyurethane prepolymer and a specified polyorganosiloxane together with a polymerization catalyst. Fibers constituting the structure are entirely covered by urethane/organosiloxane copolymer film having an elongation at break of at least 200%, a tensile recovery at 100% elongation of at least 70%, a tensile strength of 1-50 kg./cm.<sup>2</sup> and a hardness of 5-60°.

This invention relates to improved fibrous structures and a novel manufacture thereof. More particularly, it relates to fibrous structures having voluminous hand, durable elasticity, excellent anti-pilling property, shrink-proofness, crease resistance, light durability, heat resistance (melt-proofness), elastic property, mechanical properties, solvent resistance, etc., and to a novel treating process in manufacture thereof.

By the term "fibrous structures" used throughout the specification and claims, is meant structures or compositions consisting of or comprising fibers, such as staples, filaments, yarns, strings, strands, ropes, knitted goods, woven fabrics, non-woven fabrics, tufted fabrics, made-up clothes and the like.

Heretofore, it has been well-known in the art to improve water-proofness, water-repellency or the like of natural or synthetic fibrous structures by treating them with a solution or emulsion of silicone resin or polyurethane resin. Such a conventional treatment with silicone resin alone can impart superior water-proofing effect and water-repellent effect but however, it gives an undesirable hand of waxy feeling to the structure and besides the finished products are not provided with excellent anti-pilling property, light durability, shrink-proofness and crease resistance having durability enough to withstand washing. On the other hand, the method for treating with a solution or emulsion of polyurethane resin can impart fairly good crease resistance, anti-pilling property and voluminous hand to the structure, but however, it is difficult to maintain the said properties for a long time because of their poor durabilities for wash and light exposure.

There has also been proposed a method for treating fabrics with a mixture of polyurethane and polysiloxane for the purpose of producing water-proof cloths.

## 2

The above mentioned method may also impart good water-proofness and water-repellency to the cloths but those properties are not maintained for a long time owing to the lack of washing durability, light durability and heat resistance, as in the case of the above-described conventional process.

In order to overcome all the above difficulties or drawbacks, we, the inventors have made an extensive and systematic investigation on a finishing process for obtaining 10 a fibrous structure having unique hand together with the above-mentioned excellent performances and eliminated the tendency of pilling and slippage of fibers in the structure. As a result, we have accomplished the present invention on the basis of the fact that excellent effects are 15 attainable when a block copolymer as specified herein-after of a polyorganosiloxane diol and a polyurethane prepolymer is applied to and fixed on the surface of fibers constituting the fibrous structure.

Namely, an object of the present invention is to provide 20 fibrous structures with unique, voluminous hand, durable elasticity and excellent crease resistance and shrink-proofness.

Another object of the invention is to provide a method 25 for manufacturing easily and economically on an industrial scale fibrous structures having unique, voluminous hand, durable elasticity and excellent crease resistance and shrink-proofness.

A further object is to obtain fibrous structures having 30 improved light durability, heat resistance especially melt-proofness and solvent resistance.

Other objects will be apparent from the following detailed description of the invention.

The first feature of the present invention is a fibrous structure having elastic, good hand and excellent physical 35 properties which comprises fibers constituting the fibrous structure having 0.1 to 10% by weight based on said fibers of a continuous film homogeneously adhered thereto, said film consisting of a block copolymer of a polyurethane prepolymer and a polyorganosiloxane comprising predominantly a polyorganosiloxane diol, said film having an elongation at break of at least 200%, a tensile recovery at 100% elongation of at least 70%, a tensile strength of 1-50 kg./cm.<sup>2</sup> and a hardness of 5-60°.

The second feature of this invention resides in a method 45 of producing a fibrous structure having elastic, good hand and excellent physical properties which comprises sequential steps of applying homogeneously to a fibrous structure a non-aqueous organic solvent solution of a mixture comprising 10 to 1 part of a polyurethane prepolymer having 50 an —NCO group content of 1.0 to 3.0% by weight and an average molecular weight of 3,000 to 50,000 and 1 to 10 parts of a polyorganosiloxane comprising predominantly polyorganosiloxane diol having a viscosity at 25° C. in 15% trichloroethylene solution of 1,000-100,000 centistokes, together with a polymerization catalyst in an amount of 0.1 to 10% by weight based on 55 said structure of polymer solids and subsequently subjecting said structure to a heat treatment of 50 to 200° C. to complete the block copolymerization reaction of the 60 said applied polyurethane prepolymer and polyorganosiloxane, whereby a resultant block copolymer is fixed onto the fibers.

The said block copolymer fixed in the improved fibrous structure of the present invention is produced 65 by polyaddition reaction between —NCO groups of the

polyurethane prepolymer and hydroxyl groups of the polyorganosiloxane diol, and therefore, the obtained copolymer differs remarkably from a polyurethane resin or organosiloxane high polymer alone or a mixture thereof in molecular structure, solubility in an organic solvent, light durability, heat resistance, elastic properties, etc., and especially is remarkably improved in organic solvent resistance, heat resistance and light durability as compared with a mixture thereof. Particularly with respect to the organic solvent resistance, the block copolymer is substantially absolutely insoluble in an organic solvent and does not even swell therein. Therefore, the fibrous structure of the invention is much superior to the conventional fibrous structures having polyurethane resin or polyorganosiloxane alone or a mixture thereof fixed thereon in light durability, anti-pilling property, heat resistance, shrink-proofness, crease resistance, elastic properties, etc., and also is capable of maintaining these properties for a long period of time because of its good durability for laundering.

The said copolymer formed and fixed in a fibrous structure is essentially required to have an elongation at break of at least 200%, a tensile recovery at 100%, elongation of at least 70%, a tensile strength of 1-50 kg./cm.<sup>2</sup>, and a hardness of 5-60°. If even one of these physical properties deviates from its above specified range, the objects of the present invention are not attainable.

When the elongation at break is below 200%, the formed film is so poor in elasticity that a fibrous structure having durable crease resistance and shrink-proofness and elastic hand cannot be obtained. Accordingly, a more preferred elongation at break is in a range of 400 to 1,000%. The tensile recovery at 100% elongation is at least 70% and, more preferably at least 80%. The tensile strength must be in a range of 1-50 kg./cm.<sup>2</sup>, and is particularly preferred to be 3-20 kg./cm.<sup>2</sup>. If the tensile strength is below 1 kg./cm.<sup>2</sup>, the formed film is unsuitably brittle. The hardness is required to fall in a range between 5 and 60°, more preferably 8 to 30°. When the hardness is below 5°, the formed film is too soft and when it is above 60°, the fibrous structure as treated becomes undesirably rough and hard, and in either case, the hand of the structure is impaired.

In addition to the above, the amount of the said copolymer fixed to the fibrous structure is an important factor. According to the invention, 0.1 to 10% by weight based on the structure of the copolymer of polyorganosiloxane diol and polyurethane prepolymer having the physical properties as described hereinbefore is required to be applied to a fibrous structure, but in practical use, a range of 0.2 to 3% by weight is more preferable. The effect of the invention is small when the fixed amount is below 0.1% by weight, while the bulkiness and touch feeling are undesirably degraded when same is in excess of 10% by weight.

The polyorganosiloxane diol to be employed in this invention is a polysiloxane having both terminal hydroxyl groups and a viscosity at 25° C. in 15% trichloroethylene solution of 1,000 to 100,000 centistokes, which is, for instance, represented by the general formula:



wherein R and R' denote the same or different alkyl, aryl, aralkyl or alkenyl groups having a carbon atom number of 1 to 18, —CH=CH<sub>2</sub>, —CH<sub>2</sub>—CH<sub>2</sub>—CF<sub>3</sub>,



—NCO, —OH, —OCH<sub>3</sub> or the like. Among the polymers represented by the above general formula, dimethylpolysiloxane diol, diethylpolysiloxane diol, methyl-phenylpolysiloxane diol, diphenylpolysiloxane diol and  $\gamma$ -cyano-propyl-methylpolysiloxane diol are particularly preferred.

Above all, the most preferred is dimethylpolysiloxane

diol. Viscosity at 25° C. in 15% trichloroethylene solution of the said polyorganosiloxane diol to be employed in the invention is in a range of 1,000 to 100,000 centistokes, more preferably 5,000 to 50,000 centistokes. When it is below 1,000 centistokes, the said block copolymer having the above described physical properties cannot be produced, with no effect of improvement.

The polyurethane prepolymer to be employed in this invention may be any kind of polyurethane prepolymer having both terminal isocyanato groups and urethane or urea groups in the main molecular chain thereof. Such a prepolymer may be produced by reaction between an active hydrogen-containing compound and an isocyanato group-containing compound. As an organic diisocyanate which is employable to make the prepolymer, there may be mentioned, for example, 1,5-naphthylene diisocyanate, 4,4'-diphenyl-methane diisocyanate, 2,6-tolylene diisocyanate, 2,4-tolylene diisocyanate, methylene-bis-(4-phenyl isocyanate), metaphenylen diisocyanate, paraphenylen diisocyanate, diphenylmethane-3,3'-dimethyl - 4,4' - diisocyanate, xylylene diisocyanate, cyclohexylene diisocyanate, 1,6-hexamethylene diisocyanate, dimethyl diisocyanate, 4,4'-dicyclohexylmethane diisocyanate, methylcyclohexylene diisocyanate and the like. As an active hydrogen-containing compound which is employable to form long chain segment, a diol having substantially linear structure is often used and a triol or polyol having an inactive side groups such as an alkyl, alkenyl, alkaryl or aralkyl group may also be used. As a triol, for example, glycerine-propyleneoxide adduct may be employed. Preferred diols include polyalkyleneoxide glycols such as poly-1,2-propyleneoxide glycol, polyethyleneoxide glycol, ethyleneoxide-propyleneoxide copolymer glycol or the like produced from glycols as a raw material. Those diols have preferably a molecular weight of not more than 5,000.

Physical properties of the polyurethane prepolymer to be employed are important factors for forming the said tough copolymer as obtained by efficient copolymerization of the said prepolymer with the polyorganosiloxane diol under practical heat-treatment conditions.

The present inventors have investigated an interrelation between the polyurethane prepolymer and the block copolymer obtainable therefrom by copolymerization with the polyorganosiloxane diol and have found that it is necessary to use a high molecular weight prepolymer having an average molecular weight of 3,000 to 50,000, preferably 10,000 to 25,000 and an isocyanato group content of 1.0 to 3.0% by weight, preferably 1.5 to 2.5% by weight. When the average molecular weight of the said polyurethane prepolymer is less than 3,000, it is not possible to form the block copolymer of the physical properties as described before, while if it is more than 50,000, the copolymerization reaction does not progress easily. When the isocyanato group content is less than 1.0% by weight, the copolymerization reaction proceeds with difficulty, and when it is more than 3.0% by weight, the objects of the invention cannot be attained because the block copolymer having the above-defined physical properties cannot be formed.

In order to obtain the best results, the mixing ratio (copolymerization ratio) of polysiloxane diol and polyurethane prepolymer, which is also an important factor, should fall within the range of 10:1 to 1:10 by weight, outside which range there is formed no blocked copolymer having such physical properties as described above and accordingly no satisfactory improvement of the fibrous structure can be made. Namely, when the ratio of the polyurethane prepolymer to the polyorganosiloxane diol is above the upper limit of the range, the copolymer formed is unpreferably liable to be discolored into yellowish shade upon exposure to heat or light and the weather durability is remarkably degraded as compared with that of the non-treated fibrous structure. Within the above

range of mixing ratio, as the ratio of the polyurethane prepolymer increases, the hand durability for laundering and anti-pilling durability are increased. On the other hand, as the ratio of the polyorganosiloxane diol is increased, the waxy feeling is increased. When the two are employed in an equivalent amount, especially excellent elastic properties and crease resistance may be imparted. However, the most preferred mixing ratio of the two is in a range of 10:2 to 2:10, in view of the objects of the present invention.

Though the above-described many excellent effects may be attained by block copolymerizing the polyorganosiloxane diol and polyurethane prepolymer in a mixing ratio of 1:10 to 10:1 as explained hereinabove, the copolymerization may also be conducted in the coexistence of a specified amount of an alkylhydrogenpolysiloxane to form a terpolymer constituted by the polyurethane prepolymer, polyorganosiloxane diol and alkylhydrogenpolysiloxane on a fibrous structure. Thus, it was found that the water-repellency of the said fibrous structure is further enhanced thereby. The amount of the said alkylhydrogenpolysiloxane which may be added is at most 20% by weight, especially preferably in a range of 5 to 10% by weight, based on the polyorganosiloxane diol. When the addition amount is below 5% by weight, the heat resistance and water-repellency are enhanced only a little and when it is more than 20% by weight, it is not preferred as the formed copolymer film is brittle and its tensile strength is degraded.

As a preferable alkylhydrogenpolysiloxane, there may be mentioned, for example, methylhydrogenpolysiloxane, ethylhydrogenpolysiloxane, butylhydrogenpolysiloxane and the like, among which methylhydrogenpolysiloxane is most preferred. The viscosity of the alkylhydrogenpolysiloxane is preferred to be not more than 1,000 centistokes, more preferably 5 to 50 centistokes.

In the practice of the present invention, the amount of the said block copolymer fixed on a fibrous structure is also important. Namely, a mixture having a specified mixing ratio as described above of polyorganosiloxane diol and polyurethane prepolymer or a mixture further containing alkylhydrogenpolysiloxane must be applied to the fibrous structure in an amount ranging from 0.1 to 10% by weight based on the fibrous structure.

In this case, if it is below 0.1% by weight, the treating effect is insufficient and on the other hand, if it is more than 10% by weight, the bulkiness, touch feeling, etc. are unpreferably degraded. The most preferred applying amount is in a range of 0.2 to 6% by weight.

According to the invention, in order to promote the copolymerization reaction between the polyurethane prepolymer and the polyorganosiloxane diol or between them and the alkylhydrogenpolysiloxane, a polymerization catalyst is employed. As suitable polymerization catalysts there may be employed organometallic compounds exemplified by dibutyl-tin-dilaurate, dibutyl-tin-dioctoate, dibutyl-tin-octylmaleate laurate, dibutyl-tin-succinate, stannous octoate, dibutyl-tin-diethylhexoate, and tin chelated compounds which are non-limitative. The said catalysts may be used alone or in combination. The amount of the polymerization catalyst to be added is normally in a range of 1 to 30% by weight, preferably 3 to 10% by weight, based on the polyorganosiloxane diol.

In addition to the said polymerization catalyst, a primer may also be employed in order to enhance the adhesiveness of the formed block copolymer to a fibrous structure. As such a primer, there may be employed, for example, silane, isocyanate, alkoxysilanes, silane acetates, vinyltrichlorosilane, vinyl-tris-( $\beta$ -methoxy-ethoxy)-silane,  $\beta$ -(3,4-epoxycyclohexyl)-ethyl-trimethoxysilane,  $\gamma$ -glycidoxyl-propyl-trimethoxy-silane,  $\gamma$ -metacrylopropyl-trimethoxysilane or the like. These are added usually in an amount of not more than 15% by weight of the polyorganosiloxane diol.

In the treatment of a fibrous structure according to the invention, a treating solution prepared by dissolving a specific amount of polyurethane prepolymer and polyorganosiloxane diol, or a mixture thereof with alkylhydrogenpolysiloxane, in a non-aqueous, organic solvent as set forth hereinafter and, if required, further adding a catalyst and a primer thereto, is employed and is applied appropriately to a fibrous structure by means of immersion, padding, spraying, gravure coating, etc. in an amount as required. The fibrous structure impregnated with the treating solution is subsequently led into a heat-treatment apparatus held at a desired temperature, and subjected to heating to form and fix the said block copolymer therein after completion of the copolymerization reaction.

Here, the temperature for heat treatment correlates with the treating period of time, depending on the natures of the fibrous structure and the block copolymer and fixed amount of the copolymer. The treatment may be conducted at 50 to 200° C., preferably at 100 to 160° C. for 30 seconds to 20 minutes. At a temperature below 50° C., a copolymer having the required physical properties cannot be produced or it is necessary to conduct a treatment for a disadvantageously long time. A temperature above 200° C. is not preferred since the treated fibrous structure is likely to be discolored.

As a non-aqueous, organic solvent employed for the said treating solution, for example, toluene, benzene, xylene, industrial gasoline, tetrachlorocarbon, chloroform, dichloroethane, perchloroethylene, trichloroethylene, methylene chloride or the like are preferred. Each ingredient for copolymerization dissolved in the said solvent may wet and impregnate homogeneously inside and on the surface of the fibrous structure by their rapid permeation and diffusion therethrough after being applied. Also at the drying step after elimination of the solvent, the said solvent evaporates so rapidly as compared with water that there occurs no shift of a copolymer on a fibrous structure and the homogeneous, tough block copolymer is formed in situ on the fibrous structure by completion of the block copolymerization reaction on heat treatment.

The thus produced and fixed copolymer in the fibrous structure acts as a member of fibrous texture, and therefore, the treated fibrous structure exhibits, as a whole, excellent tensile elasticity and compressive elasticity against mechanical stress, and much greater crease resistance as compared with a polyurethane or polyorganosiloxane elastomer used alone or mixtures thereof and prevents pilling formation and slippage due to polyorganosiloxane elastomer. It is noticeable that the treated fibrous structure exhibits high elasticity and at the same time holds its friction coefficient well by compensating the low friction coefficient of a polyorganosiloxane component (of the copolymer) for the high friction coefficient of a polyurethane component and that elastic finished articles having various unique hands may be manufactured by varying the mixing ratio of the polyorganosiloxane diol to the polyurethane prepolymer. It is more significant that an improvement has been made owing to block copolymerization as described above, namely, the yellowing or degradation in light durability of a fibrous structure which usually resulted from finishing with a polyurethane homopolymer prepared from a polyurethane prepolymer alone has been completely eliminated by block copolymerization of a polyorganosiloxane diol therewith. Furthermore, synthetic resin finishing of fibrous structures heretofore practised is accompanied by a drawback of fixing cross-over contacts in the texture of cloth, and so the stretchability of fibrous structures such as knitted goods is inevitably reduced thereby. However, according to the invention there is only a little concentration of the copolymer on cross-over contacts in the texture since a non-aqueous organic solvent is employed, and even if the copolymer is concentrated, the stretching

characteristic is not impaired since the copolymer itself has high tensile elasticity.

The method of the present invention displays its best effect in the treatment of knitted goods and gives an excellent effect also in the treatment of yarns, woven fabrics, non-woven fabric, made-up clothes, carpets or the like. Particularly, the shrink-proof effect obtained by the present invention assures dimensional stability of the fibrous structure and the high degree of heat resistance leads to an improvement in heat melting characteristic which was hitherto a drawback of polyamide and polyester fibers. Such defects specific in synthetic fibers such as, for example, clothes made of thin textiles such as nylon taffeta are easily melted by lighted tobacco, etc. to make holes therein, or traces of needles by sewing machines are improved.

Textile finished with polyorganosiloxane elastomer alone are so slippery that disadvantages are encountered in spreading and cutting, but on the contrary, there is no such a problem in the fibrous structure of the present invention.

Another advantage of the fibrous structure of the invention is that piece dyeing thereof is possible. This is one of the prominent features that have never been seen heretofore until the present invention was accomplished, where the said copolymer formed in the method of this invention possesses eminent elasticity, shrink-proofness and hot water resistance.

The fibrous structure obtained according to the process of the present invention is remarkably excellent in durability, in particular durability for laundering and dry cleaning since the copolymer, which is remarkably improved by the block copolymerization reaction with regard to solvent resistance, water resistance, light durability, heat resistance, etc., is firmly bonded and fixed to the texture of the said fibrous structure. On the contrary, a polymer film formed by treating a polyorganosiloxane diol which will be polymerized and polyurethane resin (dead polyurethane polymer) together with a polymerization catalyst in a similar manner to the present invention is poor in resistance against mechanical stress, organic solvents, detergents, etc. and physical properties such as elasticity, crease resistance, etc. as well as durability for laundering and dry cleaning. These facts will be apparent from the examples as mentioned hereinafter.

The method of the present invention is applicable to all kinds of fibrous structures such as yarns, knitted and woven fabrics, non-woven fabrics, made-up clothes or the like. The yarn includes filament, spun yarn and bulky yarn. The bulky yarn includes those processed by a false-twisting method, twisting and untwisting method with Italian twister, stuffing box method, knitting and deknitting method, knife edging method, air-jet method, etc. and may be treated with prepolymer prior to or after those texturizing processes.

The fibers to be treated include natural fibers such as wool, silk, cotton, linen or the like, synthetic fibers comprising, for example, polyester, polyamide, polyurea, polyacrylonitrile, polyvinyl chloride or the like and regenerated fibers such as viscose rayon, cupro-rayon or the like.

The present invention is further illustrated by the following non-limitative examples. In the examples, the term "part" means "part by weight." The methods of measuring crease resistance, elongation at break, compressive elasticity (degree of compression, degree of elasticity), tensile elasticity (load for elongation degree of elasticity), anti-pilling property and melting-proofness, and conditions of laundering and dry cleaning are as follows:

#### Crease resistance

Measurement is made according to JIS (Japanese Industrial Standard) L-1079-5.22.2 B method.

#### Compressive elasticity

Four sheets of cloth are superimposed on each other, the total thickness ( $t$  mm.) after a load of 10 g./cm.<sup>2</sup> is applied thereto for one minute is measured, then the thickness ( $t_1$  mm.) after another load of 30 g./cm.<sup>2</sup> is applied thereto for one minute is measured and the thickness ( $t_2$  mm.) after standing for another one minute under no load is determined. Thus the degree of compression and the degree of resiliency are expressed by the following equations:

$$\text{Degree of compression (percent)} = \frac{t-t_1}{t} \times 100$$

$$\text{Degree of resiliency (percent)} = \frac{t_2-t_1}{t-t_1} \times 100$$

#### Tensile elasticity

(1) Load for elongation.—The load (g) required for a specimen of 10 cm. long and 2.5 cm. wide to be stretched on an Instron tension tester at a rate of 10 cm./min. up to a predetermined elongation is measured.

(2) Degree of elasticity.—A load of 500 g. is applied in the similar manner to (1) above, when the length ( $l_1$  cm.) is measured. After loading for a minute followed by further standing for a minute under no load, the length ( $l_2$  cm.) is measured. The original length of the specimen ( $l_0$  cm.) Thus the degree of elasticity is represented by the following equation:

$$\text{Degree of elasticity (percent)} = \frac{l_1-l_2}{l_1-l_0} \times 100$$

#### Tearing strength

Measured according to JIS L-1079-5.14 Tear strength C method.

#### Pilling test

Measured according to JIS L-1076 (1967) A method (by means of ICI type tester)

#### Melt-proofness test

A cigarette just lit is laid on the specimen under conditions of a relative humidity of 65% and temperature of 20° C. and the time required till it melts and makes a hole is measured.

#### Laundering

(1) Mixed spun yarn broad-cloth of polyester/cotton.—Measured according to JIS L-1042 F-3 shrinking test of Sanforized poplin of polypropylene/rayon.

(2) Wool.—Measured according to the IWS test method.

#### Dry cleaning

Carried out continuously for 3 hours at 25° C. using 50 time bath of perchloroethylene according to AATCC method.

#### EXAMPLE 1

A double jersey fabric (the length extended in the wale direction was 70 mm./50 courses) knitted with a false-twist textured nylon-6 yarn of 70 denier of 18 filaments/2 ply was scoured at 70° C. for 20 minutes in a 30 times bath containing 1 g./l. each of an anionic surfactant and of soda ash, dried (density, wale: 30/inch; course: 45/inch), padded with solution of the under-mentioned composition (pick-up: 140%), dried again at 80° C. and then was heat-treated at 150° C. for 2 minutes.

The resultant fabric (density, wale: 37/inch; course: 45/inch) contained 3.1% by weight of copolymer exhibited a favourable voluminous hand of elasticity, excellent elastic recovery from elongation, desirable durability for washing, crease resistance, anti-pilling property and melt-proofness.

## Composition of treating solution

Parts

|                                                                                                                                                                                                                                                       |      |    |
|-------------------------------------------------------------------------------------------------------------------------------------------------------------------------------------------------------------------------------------------------------|------|----|
| Dimethylpolysiloxane diol (viscosity at 25° C. of 15% trichloroethylene solution: 20,000 centistokes)                                                                                                                                                 | 2    | 5  |
| Polyurethane prepolymer having an average molecular weight of 18,000 and an isocyanato group content of 1.8% by weight obtained by 6 mols of polypropyleneether glycol (MW: 2,000), 12 mols of tolylene diisocyanate and 1 mol of polypropylene triol | 1    | 10 |
| Dibutyl-tin-dilauroate (polymerization catalyst)                                                                                                                                                                                                      | 0.15 | 15 |
| N-(trimethoxypropyl) ethylenediamine (primer)                                                                                                                                                                                                         | 0.15 | 15 |
| Trichloroethylene (solvent)                                                                                                                                                                                                                           | 97   | 15 |

The above treating solution was treated in the similar manner to the above process and there was formed a film (thickness: 1 mm.) which exhibited the following physical properties:

Elongation at break: 510%  
 Elastic recovery at 100% elongation: 82%  
 Tensile strength: 6 kg./cm.<sup>2</sup>  
 Hardness: 12°

The result is shown in Table 1.

TABLE 1

|                           | Tensile elasticity |                   |               |                   | Compressive elasticity (percent) |      |               |      | Anti-pilling property (rating) | Hand | Melt-proofness (sec.)    |  |  |  |
|---------------------------|--------------------|-------------------|---------------|-------------------|----------------------------------|------|---------------|------|--------------------------------|------|--------------------------|--|--|--|
|                           | Before washing     |                   | After washing |                   | Before washing                   |      | After washing |      |                                |      |                          |  |  |  |
|                           | L.<br>(g.)         | D.E.<br>(percent) | L.<br>(g.)    | D.E.<br>(percent) | D.C.                             | D.E. | D.C.          | D.E. |                                |      |                          |  |  |  |
| Untreated                 | 152                | 73                | 154           | 71                | 19                               | 71   | 22            | 94   | 4.5                            | 3    | 31                       |  |  |  |
| Article of this invention | 158                | 96                | 160           | 94                | 22                               | 96   | 21            | 94   | 5                              | 3.5  | Scooping, bulky feeling. |  |  |  |
| Control (A)               | 140                | 94                | 145           | 89                | 21                               | 94   | 18            | 88   | 5                              | 1.5  | Waxy feeling.            |  |  |  |
| Control (B)               | 165                | 90                | 162           | 88                | 19                               | 92   | 19            | 89   | 2                              | 4    | A little hard.           |  |  |  |
| Control (C)               | 168                | 89                | 150           | 80                | 19                               | 89   | 19            | 83   | 3                              | 3    | do.                      |  |  |  |

NOTE.—L=Load; D.E.=Degree of elasticity; D.C.=Degree of compression.

In Table 1, the compositions and conditions of the controls are as follows:

## Control A

Parts

|                                           |      |
|-------------------------------------------|------|
| Dimethylpolysiloxane diol same as above   | 3    |
| Dibutyl-tin-dilauroate                    | 0.15 |
| N-(trimethoxysilylpropyl) ethylenediamine | 0.15 |
| Trichloroethylene                         | 97   |

The treating solution comprising the above ingredients was applied similarly to the fabric and fixed in a solid amount of 4.2% by weight to the fabric.

## Control B

The solution consisting of 3 parts of polyurethane prepolymer same as above and 97 parts of trichloroethylene was applied similarly and fixed in a solid amount of 4.2% by weight to the fabric.

## Control C

Parts

|                                                                                      |      |
|--------------------------------------------------------------------------------------|------|
| Dimethylpolysiloxane diol                                                            | 1.5  |
| Dibutyl-tin-dilauroate                                                               | 0.15 |
| N-(trimethoxysilylpropyl) ethylenediamine                                            | 0.15 |
| Parapren (the trade name of polyurethane resin manufactured by Hodogaya Kagaku K.K.) | 1.5  |

The solution consisting of the above ingredients was ap-

plied similarly and fixed in a solid amount of 4.2% by weight to the fabric.

## 10

The treated article of the invention was dyed homogeneously in the composition having a bath ratio of 30:1 of 1.2% by weight of Kitten Fast Violet R (an acidic dyestuff manufactured by Ciba Ltd.) and 1% by weight of Liogen P (a surfactant manufactured by Sandoz A.G.), with no degradation of physical properties.

## EXAMPLE 2

A fabric of double half tricot knitted with a raw silk yarn of 21 denier of 7 filaments/2 ply was scoured at 100° C. for one hour in a 40 times bath containing 3 g./l. of potash soap, then subjected to a beam-dyeing in a bath containing 10% by weight of Direct Deep Black EAC (direct dyestuff manufactured by Ciba Ltd.), and was dried at 100° C. on a tenter-drier (density, wale 42/inch; course: 46/inch). The thus dried fabric was immersed in the solution of the composition as mentioned hereafter, squeezed at a pickup of 80%, dried again at 80° C. and then heat-treated at 120° C. for 2 minutes. The resultant fabric (density, wale: 42/inch; course: 45.5/inch) contained 1.6% of copolymer and exhibited excellent crease resistance and elasticity, so that it was suitable for lady's wear and gloves.

TABLE 2

|  | Composition of treating solution                                                                                                                                                                                                                                                                                                                                                       |     |                                                           |     | Parts |
|--|----------------------------------------------------------------------------------------------------------------------------------------------------------------------------------------------------------------------------------------------------------------------------------------------------------------------------------------------------------------------------------------|-----|-----------------------------------------------------------|-----|-------|
|  |                                                                                                                                                                                                                                                                                                                                                                                        |     |                                                           |     |       |
|  | Dimethylpolysiloxane diol (viscosity at 25° C. of 15% trichloroethylene solution: 11,000 centistokes)                                                                                                                                                                                                                                                                                  | 1.2 | Methyl - hydrogenpolysiloxane (viscosity: 18 centistokes) | 0.3 |       |
|  | Polyurethane prepolymer having an isocyanato group content of 2.0% by weight and an average molecular weight of 23,000 obtained from 1 mol of polyester glycol (MW: 2,000) which was obtained from the reaction between a 80:20 mixture of polypropyleneether glycol and propylene glycol and adipic acid, 5 mols of 4,4'-diphenylmethane diisocyanate and 0.02 mol of 1,4-butane diol | 0.5 |                                                           |     |       |
|  | Dibutyl-tin-octylmaleate laurate (catalyst)                                                                                                                                                                                                                                                                                                                                            | 0.1 | γ-Glycidoxypropyl-trimethoxysilane (primer)               | 0.1 |       |
|  | 1,1,1-trichloroethane (solvent)                                                                                                                                                                                                                                                                                                                                                        | 98  |                                                           |     |       |

A film prepared from the above solution in the similar manner to Example 1 exhibited the following physical properties:

Elongation at break: 620%  
 Elastic recovery at 100% elongation: 75%  
 Tensile strength: 10 kg./cm.<sup>2</sup>  
 Hardness: 21°

The result is shown in the following Table 2.

TABLE 2

|                           | Tensile elasticity  |                   |                    |                   | Crease resistance   |        |                    |        | Parts                    |  |
|---------------------------|---------------------|-------------------|--------------------|-------------------|---------------------|--------|--------------------|--------|--------------------------|--|
|                           | After just finished |                   | After dry cleaning |                   | After just finished |        | After dry cleaning |        |                          |  |
|                           | L.<br>(g.)          | D.E.<br>(percent) | L.<br>(g.)         | D.E.<br>(percent) | Wale                | Course | Wale               | Course |                          |  |
| Untreated                 | 142                 | 59                | 143                | 57                | 57                  | 58     | 58                 | 57     |                          |  |
| Article of this invention | 152                 | 93                | 150                | 91                | 80                  | 81     | 79                 | 81     | Soft, scrooping feeling. |  |
| Control (A)               | 125                 | 92                | 128                | 86                | 78                  | 79     | 77                 | 78     | Much waxy feeling.       |  |
| Control (B)               | 162                 | 88                | 155                | 87                | 69                  | 69     | 68                 | 69     | A little hard.           |  |
| Control (C)               | 145                 | 83                | 144                | 65                | 80                  | 81     | 68                 | 67     | Do.                      |  |

The controls (A), (B) and (C) in Table 2 were produced in a similar manner to Example 1 wherein the control (A) was fixed by the above polyorganosiloxane prepolymer in a pick-up of 1.6%, the control (B) by the above polyurethane prepolymer in a pick-up of 1.6% and the control (C) by a pick-up of 0.8% each of the above polyorganosiloxane prepolymer and the polyurethane resin in the control (C) of Example 1.

## EXAMPLE 3

A twill of acrylic spun-yarn (warp: 1/50 count; filling: 1/32 count, density, warp: 86/inch; filling: 80/inch) was padded with the following solution of the composition (pick-up: 60%), dried at 80° C. and then heat-treated at 170° C. for 30 seconds. The thus-obtained fabric contained 1.8% by weight of copolymer and exhibited soft, voluminous, drape, elastic hand and superior crease resistance and anti-pilling property. The fabric was not deformed by repeated wearing and washing.

## Composition of treating solution

|                                                                                                                                                                                                                                                                                                                                                                                    | Parts |
|------------------------------------------------------------------------------------------------------------------------------------------------------------------------------------------------------------------------------------------------------------------------------------------------------------------------------------------------------------------------------------|-------|
| Dimethylpolysiloxane diol (viscosity at 25° C. of 15% trichloroethylene solution: 30,000 centistokes) -----                                                                                                                                                                                                                                                                        |       |
| Polyurethane prepolymer having an isocyanato group content of 2.6% by weight and an average molecular weight of 15,300 made from 1 mol of polycaprolactone diol (MW: 1,300) which was obtained by the reaction of $\epsilon$ -caprolactone, methyl- $\epsilon$ -caprolactone and methyl-diethanolamine, 2 mols of hexamethylene diisocyanate and 0.03 mol of 1,4-butane diol ----- |       |
| $\beta$ -(3,4-epoxycyclohexyl) ethylmethoxysilane (primer) -----                                                                                                                                                                                                                                                                                                                   | 0.1   |
| Stannous octoate (catalyst) -----                                                                                                                                                                                                                                                                                                                                                  | 0.1   |
| Perchloroethylene (solvent) -----                                                                                                                                                                                                                                                                                                                                                  | 97    |

The film prepared from the above solution exhibited the following physical properties:

Elongation at break: 600%

Elastic recovery at 100% elongation: 73%

Tensile strength: 5 kg./cm.<sup>2</sup>

Hardness: 24°

The result is shown in Table 3.

manner to Example 1 wherein the control (A) was applied with 1.8% of the above polyorganosiloxane prepolymer, the control (B) with 1.8% of the above polyurethane prepolymer, and the control (C) with 0.9% of the above polyorganosiloxane prepolymer together with 0.9% of polyurethane resin (Krisbon 7667 manufactured by Nippon Reichhold K.K.).

## EXAMPLE 4

10 Woolen fabric knitted of worsted yarn of 1/44 count (density, wale: 39/inch; course: 34/inch) was relaxed by hot-tumbling to the density of wale: 38/inch; course: 35/inch, padded with the following solution of the composition (pick-up: 85%), dried at 70° C. and then heat-treated at 120° C. for 10 minutes. The obtained fabric (density, wale: 38/inch; course: 35.5/inch) contained 2.6% by weight of copolymer, showed superior voluminous hand of elasticity and drapeness as compared with the under-mentioned (A) or (B) each alone, and exhibited excellent tensile recovery, and shrink-proofness and crease resistance of durability for washing.

## Composition of treating solution

|                                                                                                                                                                                                                                                                                                                          | Parts |
|--------------------------------------------------------------------------------------------------------------------------------------------------------------------------------------------------------------------------------------------------------------------------------------------------------------------------|-------|
| 1 25 Dimethylpolysiloxane diol (viscosity at 25° C. of 15% trichloroethylene solution: 22,000 centistokes) -----                                                                                                                                                                                                         | 0.8   |
| 30 Methylhydrogenpolysiloxane (viscosity 20 centistokes) -----                                                                                                                                                                                                                                                           | 0.2   |
| 3 35 Polyurethane prepolymer having an isocyanato group content of 2.0% by weight and an average molecular weight of 4,180 obtained from a reaction product of 1 mol of $\epsilon$ caprolactone diol (MW: 1,740) 1.5 mols of 4,4'-dicyclohexylmethane diisocyanate, and 1 mol of 4,4'-diphenylmethane diisocyanate ----- | 2.2   |
| 40 Dibutyl-tin-diethylhexoate (catalyst) -----                                                                                                                                                                                                                                                                           | 0.15  |
| 45 Methyleneethylketone (solvent) -----                                                                                                                                                                                                                                                                                  | 97    |

The film prepared from the treating solution in a similar manner to Example 1 exhibited the following physical properties:

Elongation at break: 560%

Elastic recovery at 100% elongation: 80%

Tensile strength: 5.2 kg./cm.<sup>2</sup>

Hardness: 15°

TABLE 3

|                                 | Compressive elasticity (percent) |      |               |      | Crease resistance (percent) |         |               |         | Antipilling property (rating) |         |
|---------------------------------|----------------------------------|------|---------------|------|-----------------------------|---------|---------------|---------|-------------------------------|---------|
|                                 | Before washing                   |      | After washing |      | Before washing              |         | After washing |         | Before                        | After   |
|                                 | D.C.                             | D.E. | D.C.          | D.E. | Warp                        | Filling | Warp          | Filling | washing                       | washing |
| Untreated -----                 | 20                               | 83   | 19            | 81   | 83                          | 83      | 81            | 82      | 2                             | 1       |
| Article of this invention ----- | 22                               | 93   | 21            | 92   | 91                          | 93      | 91            | 92      | 4                             | 3       |
| Control (A) -----               | 23                               | 90   | 22            | 86   | 90                          | 88      | 86            | 85      | 1                             | 1       |
| Control (B) -----               | 22                               | 88   | 21            | 85   | 88                          | 87      | 85            | 84      | 4                             | 3       |
| Control (C) -----               | 21                               | 87   | 20            | 82   | 87                          | 86      | 84            | 82      | 2                             | 1       |

The controls (A), (B) and (C) were made in a similar

The result is shown in Table 4.

TABLE 4

|                                 | Tensile elasticity  |                |                    |                | Compressive elasticity |      |                    |      | Shrinkage by washing (percent) | Felting tendency | Hand          | Light durability (rating) |  |  |  |  |
|---------------------------------|---------------------|----------------|--------------------|----------------|------------------------|------|--------------------|------|--------------------------------|------------------|---------------|---------------------------|--|--|--|--|
|                                 | Before dry cleaning |                | After dry cleaning |                | Before dry cleaning    |      | After dry cleaning |      |                                |                  |               |                           |  |  |  |  |
|                                 | L. (g.)             | D.E. (percent) | L. (g.)            | D.E. (percent) | D.C.                   | D.E. | D.C.               | D.E. |                                |                  |               |                           |  |  |  |  |
| Untreated -----                 | 165                 | 85             | 163                | 82             | 24                     | 88   | 25                 | 87   | 13                             | 15               | High          | 4                         |  |  |  |  |
| Article of this invention ----- | 175                 | 95             | 173                | 95             | 27                     | 96   | 26                 | 95   | 2                              | 1                | Slight        | 4.5                       |  |  |  |  |
| Control A -----                 | 133                 | 92             | 142                | 89             | 26                     | 94   | 25                 | 92   | 3                              | 3                | do            | Waxy feeling              |  |  |  |  |
| Control (B) -----               | 188                 | 90             | 180                | 88             | 25                     | 93   | 25                 | 91   | 2                              | 2                | do            | Hard                      |  |  |  |  |
| Control (C) -----               | 165                 | 88             | 160                | 82             | 26                     | 91   | 25                 | 87   | 8                              | 10               | A little high | A little hard             |  |  |  |  |

In Table 4, the controls (A), (B) and (C) were made in a similar manner to Example 1 wherein the control (A) was applied with 2.6% of the above polyorganosiloxane prepolymer, the control (B) with 2.6% of the above polyurethane prepolymer and the control (C) with 1.3% of the above polyorganosiloxane prepolymer together with 1.3% of the polyurethane resin (dead polymer) of Example 1.

## EXAMPLE 5

A broadcloth consisting of blend spun yarn of 65% polyester (polyethylene terephthalate) and 35% cotton

5

was scoured, bleached, fluorescent-dyed, padded with the treating solution of Example 5 (pick-up: 102%), and then heat-treated at 160° C. for 2 minutes. The thus-obtained fabric contained 1.6% of copolymer and exhibited a favourable, voluminous hand and durable

crease resistance and anti-pilling property.

The result is shown in Table 6.

TABLE 6

|                           | Crease resistance (crease recovery percent) |         |               |         |                     |         | Antipilling property (rating) |               |
|---------------------------|---------------------------------------------|---------|---------------|---------|---------------------|---------|-------------------------------|---------------|
|                           | Before washing                              |         | After washing |         | Shrinkage (percent) |         | Before washing                | After washing |
|                           | Warp                                        | Filling | Warp          | Filling | Warp                | Filling |                               |               |
| Untreated                 | 81                                          | 76.8    | 78            | 76      | 4.2                 | 3.2     | 3                             | 2             |
| Article of this invention | 88.5                                        | 86.5    | 87.5          | 86      | 1.8                 | 1.0     | 3.5                           | 3             |
| Control (A)               | 86                                          | 84.5    | 82            | 81      | 2.5                 | 1.5     | 1                             | 1.5           |

(1/40 count, density, warp: 120/inch; filling: 70/inch) was scoured, bleached, further whitened by fluorescent dye, padded with the following solution of the composition (pick-up: 110%), and then subjected to heat-treatment at 170° C. for one minute. The obtained fabric contained 1.8% by weight of copolymer and exhibited a favourable resilient, voluminous, scooping hand and excellent crease resistance and anti-pilling property.

## Composition of treating solution

|                                                                                                                                                                                                                                                                            | Parts |
|----------------------------------------------------------------------------------------------------------------------------------------------------------------------------------------------------------------------------------------------------------------------------|-------|
| Dimethylpolysiloxane diol (viscosity at 25° C. of 15% trichloroethylene solution: 18,000 centistokes)                                                                                                                                                                      | 0.6   |
| Methylhydrogenpolysiloxane (viscosity 10 centistokes)                                                                                                                                                                                                                      | 35    |
| Polyurethane prepolymer having an isocyanato group content of 1.8% by weight and an average molecular weight of 10,000 obtained from 1 mol. of polypropyleneether glycol (MW: 2,000), 2 mols of tolylene diisocyanate and 1.6 mols of polypropyleneether triol (MW: 4,000) | 1     |
| Dimethyltin-dilaurate (catalyst)                                                                                                                                                                                                                                           | 0.05  |
| n-(Dimethoxymethylsilyl propyl) ethylenediamine (primer)                                                                                                                                                                                                                   | 0.05  |
| Xylene (solvent)                                                                                                                                                                                                                                                           | 98    |

The film formed from this treating solution in a similar manner to Example 1 exhibited the following physical properties.

Elongation at break: 550%

Elastic recovery at 100% elongation: 70%

Tensile strength: 8 kg./cm.<sup>2</sup>

Hardness: 80

The result is shown in Table 5.

TABLE 5

|                           | Crease resistance (crease recovery percent) |         |               |         | Anti-pilling property (rating) |               |                           |
|---------------------------|---------------------------------------------|---------|---------------|---------|--------------------------------|---------------|---------------------------|
|                           | Before washing                              |         | After washing |         | Before washing                 | After washing | Light durability (rating) |
|                           | Warp                                        | Filling | Warp          | Filling |                                |               |                           |
| Untreated                 | 80                                          | 79      | 79            | 74      | 2                              | 1.5           | 2                         |
| Article of this invention | 87                                          | 86      | 86            | 85      | 4                              | 3             | 2                         |
| Control (A)               | 82                                          | 81      | 81            | 80      | 1                              | 1             | 2                         |
| Control (B)               | 83                                          | 82      | 81            | 81      | 4                              | 3             | 1                         |
| Control (C)               | 82                                          | 82      | 79            | 76      | 2                              | 1             | 1                         |

NOTE.—The controls were treated in a similar manner to the present invention except for employing the following treating solutions:

Control (A)—A solution containing 1.7 parts of the polyorganosiloxane prepolymer, the catalyst and 98 parts of xylene.

Control (B)—A solution containing 1.7 parts of the polyurethane prepolymer and 98 parts of xylene.

Control (C)—A solution containing 0.8 part of the polyorganosiloxane prepolymer, and the catalyst, 0.9 part of the polyurethane resin of Example 1 and 98 parts of xylene.

14  
EXAMPLE 6

A poplin woven with 40 count blend spun yarn of 50% polypropylene and 50% rayon (density, wrap: 110/inch; filling: 70/inch) was scoured, bleached, fluorescent-dyed, padded with the treating solution of Example 5 (pick-up: 102%), and then heat-treated at 160° C. for 2 minutes. The thus-obtained fabric contained 1.6% of copolymer and exhibited a favourable, voluminous hand and durable

crease resistance and anti-pilling property.

The result is shown in Table 6.

TABLE 6

|                           | Crease resistance (crease recovery percent) |         |               |         |                     |         | Antipilling property (rating) |               |
|---------------------------|---------------------------------------------|---------|---------------|---------|---------------------|---------|-------------------------------|---------------|
|                           | Before washing                              |         | After washing |         | Shrinkage (percent) |         | Before washing                | After washing |
|                           | Warp                                        | Filling | Warp          | Filling | Warp                | Filling |                               |               |
| Untreated                 | 81                                          | 76.8    | 78            | 76      | 4.2                 | 3.2     | 3                             | 2             |
| Article of this invention | 88.5                                        | 86.5    | 87.5          | 86      | 1.8                 | 1.0     | 3.5                           | 3             |
| Control (A)               | 86                                          | 84.5    | 82            | 81      | 2.5                 | 1.5     | 1                             | 1.5           |

## EXAMPLE 7

A warp-elastic fabric having a twill texture woven with false-twist textured nylon yarn (70 denier of 18 filaments/2 ply) in warp and acetate filament (150 denier of 60 filaments) in weft was applied with the treating solution of Example 4 in a pick-up of 2% of copolymer by means of spraying and heat-treated at 150° C. for 3 minutes.

The resulted fabric showed scooping, drape, voluminous hand and durable crease resistance and stretching recovery.

The untreated article made a hole on the fabric after five seconds on melt-proof test, but the treated article of the invention made no hole even after 25 seconds.

## EXAMPLE 8

Men's socks (density, wale: 29/inch; course: 43/inch) knitted with a false-twist textured nylon-6 yarn of 70 denier of 32 filament/2 ply were soaked in the treating solution of Example 2. After squeezing (pick-up: 40%), the socks were dried at 80° C. and then heat-treated at 150° C. for 2 minutes. The resulted socks after finishing treatment showed neither shrinkage nor deformation and contained 0.8% by weight of copolymer. They exhibited excellent fit and resiliency, and showed no musty feeling inherent in nylon on wearing and neither waxy feeling nor slippery feeling as in the case of the sole silicone resin finished product, so that the wearing feeling was comfortable.

## EXAMPLE 9

A double jersey fabric (the length extended in the wale direction was 65 mm./50 courses) knitted with polyester textured yarn of 110 denier of 32 filaments/2 ply was scoured, dyed with a dispersed dye, dried (density, wale:

37/inch; course: 43/inch), padded with the following treating solution of the composition (pick-up: 116%), dried again at 80° C. and then heat-treated at 170° C. for 1.5 minutes. The resulted fabric (density, wale: 36/inch; course: 44/inch) contained 2.8% by weight of copolymer and exhibited scooping touch with no waxy feeling, and excellent elastic recovery, crease resistance and anti-pilling property.

## Composition of treating solution

|                                                                                                                                                                                                                                                                     | Parts |
|---------------------------------------------------------------------------------------------------------------------------------------------------------------------------------------------------------------------------------------------------------------------|-------|
| Dimethylpolysiloxane diol containing 10 mol percent of $\gamma$ -cyanopropylmethyl siloxane unit (viscosity at 25° C. of 15% trichloroethylene solution: 5,500 centistokes)                                                                                         | 5     |
| Polyurethane prepolymer having an isocyanato group content of 2.0% by weight and an average molecular weight of 18,000 obtained from 6 mols of polypropyleneether glycol (MW: 2,000), 12 mols of tolylene diisocyanate and 1 mol of polypropylene triol (MW: 4,000) | 1.8   |
| Dibutyl-tin-dilauroate (catalyst)                                                                                                                                                                                                                                   | 0.06  |
| n - (dimethoxymethylsilylpropyl) ethylenediamine (primer)                                                                                                                                                                                                           | 0.06  |
| Trichloroethylene (solvent)                                                                                                                                                                                                                                         | 98    |

The copolymer film made from this solution is a similar manner to Example 1 showed the following physical properties:

Elongation at break: 530%

Elastic recovery at 100% elongation: 83%

Tensile strength: 18 kg./cm.<sup>2</sup>

Hardness: 12°

The result is shown in Table 7.

TABLE 7

|                                | Elastic recovery at 100% elongation in course |                |               |                |                    |                |                                |                       |                           |                    |
|--------------------------------|-----------------------------------------------|----------------|---------------|----------------|--------------------|----------------|--------------------------------|-----------------------|---------------------------|--------------------|
|                                | Before washing                                |                | After washing |                | After dry-cleaning |                | Anti-pilling property (rating) | Melt proofness (sec.) | Light durability (rating) | Hand               |
|                                | L. (g.)                                       | D.E. (percent) | L. (g.)       | D.E. (percent) | L. (g.)            | D.E. (percent) |                                |                       |                           |                    |
| Untreated.....                 | 222                                           | 75             | 218           | 73             | 220                | 74             | 2                              | 3                     | 4                         |                    |
| Article of this invention..... | 238                                           | 98             | 235           | 96             | 233                | 98             | 3.5                            | 30                    | 4                         | Scrooping touch.   |
| Control (A).....               | 205                                           | 92             | 210           | 88             | 215                | 90             | 1                              | 30                    | 4                         | Much waxy feeling. |
| Control (B).....               | 265                                           | 86             | 235           | 84             | 235                | 83             | 3.5                            | 5                     | 1                         | Hard.              |
| Control (C).....               | 230                                           | 87             | 225           | 82             | 218                | 79             | 2                              | 8                     | 1.5                       | Scrooping touch.   |

NOTE.—The controls were treated in a similar manner to the present article except for employing the following treating solution:

Control (A)—A solution containing 2.4 parts of the said silicone prepolymer, 0.12 part of the catalyst and 98 parts of trichloroethylene.

Control (B)—A solution containing 2.4 parts of the said polyurethane prepolymer and 98 parts of trichloroethylene.

Control(C)—A solution containing 1.8 parts of the said silicone prepolymer, 0.12 part of the catalyst, 0.6 part of the dead polyurethane polymer of Example 1 and 98 parts of trichloroethylene.

## EXAMPLE 10

A skein (500 g.) of a false-twist textured nylon-6 yarn of 70 denier of 18 filaments/2 ply, was immersed in the bath of treating solution of Example 4 for one minute, after which it was put into a centrifugal separator to dry up to a water content of 22% and then air-dried. The dried yarn was heat-treated at 100° C. for 20 minutes. The obtained yarn contained 0.7% of the fixed resin and exhibited such a good drapeness and elastic hand that untreated nylon-6 yarn could not obtain. The socks knitted with the treated yarn (plain stitch density, wale: 28/inch; course 41/inch) were superior in stretchability, stretching recovery and fit, showed little variation in density of stitches caused by a fluctuation of tension in the knitting process, and the knitting process was performed smoothly. On the contrary, the knitting operation in the case of the yarn treated with the sole polyurethane prepolymer was slightly difficult.

What is claimed is:

1. A method of producing a fibrous structure having elastic, good hand and excellent physical properties, comprising the sequence of steps of: applying homogeneously to a fibrous structure a non-aqueous organic solvent solution of a mixture comprising (A) 10 to 1 part of a polyurethane prepolymer having an —NCO group content of 1.0 to 3.0% by weight and an average molecular weight of 3,000 to 50,000, (B) 1 to 10 parts of a polyorganosiloxane comprising predominantly polyorganosiloxane diol having a viscosity at 25° C. in 15% trichloroethylene solution of 1,000–100,000 centistokes, and (C) a polymerization catalyst in an amount of 0.1 to 10% by weight based on the

45 solution contains also a primer selected from the group consisting of N-(trimethoxypropyl) ethylenediamine,  $\gamma$ -glycidoxypropyl-trimethoxysilane,  $\beta$  - (3,4 - epoxycyclohexyl)-ethyl-methoxy-silane, and N - (dimethoxymethylsilylpropyl) ethylenediamine, in an amount of not more than 15% by weight of said polyorganosiloxane.

9. The method as set forth in claim 1 wherein said polymerization catalyst is an organo-metallic compound selected from the group consisting of dibutyl-tin-dilauroate, dibutyl-tin-octylmaleate laurate, stannous octoate and dibutyl-tin-diethylhexoate, and its amount is 1 to 30% by weight based on said polyorganosiloxane.

10. The method as set forth in claim 9 wherein the amount of said polymerization catalyst is in a range of 3 to 10% by weight.

11. The method as set forth in claim 1 wherein the viscosity of said polyorganosiloxane diol is 5,000–50,000 centistokes.

12. The method as set forth in claim 1 wherein said average molecular weight is 10,000–25,000 and the isocyanato group content is 1.5 to 2.5% by weight.

13. The method as set forth in claim 1 wherein the proportion of polyorganosiloxane diol to polyurethane prepolymer is 2:10 to 10:2.

14. The method as set forth in claim 1 wherein the fixed amount of said copolymer is 0.2 to 6% by weight based on the fibrous structure.

15. The method as set forth in claim 1 wherein said fibrous structure is of knitted fabric.

16. The method as set forth in claim 1 wherein said heat treatment is conducted at a temperature of 100-160° C. for 30 seconds-20 minutes.

## References Cited

UNITED STATES PATENTS

|           |         |           |             |
|-----------|---------|-----------|-------------|
| 2,817,643 | 12/1957 | Altner    | 260-33.8 UB |
| 3,308,080 | 3/1967  | Haenni    | 260-33.8 SB |
| 3,562,352 | 2/1971  | Nyilas    | 117-161     |
| 3,463,662 | 8/1969  | Hodes     | 117-161     |
| 3,567,499 | 3/1971  | Klebert   | 117-161 X   |
| 3,133,891 | 5/1964  | Ceyzeriat | 117-161     |
| 3,061,567 | 10/1962 | Keil      | 117-161     |

|             |         |                 |           |
|-------------|---------|-----------------|-----------|
| 3,243,475   | 3/1966  | Reishl et al.   | 117-161 X |
| 3,246,048   | 9/1966  | Haluska         | 117-161 X |
| 3,398,043   | 8/1968  | Youngs          | 117-161 X |
| 3,419,422   | 12/1968 | Pepe            | 117-161 X |
| 5 3,450,791 | 6/1969  | Sekmakas et al. | 117-161 X |

WILLIAM D. MARTIN, Primary Examiner

M. R. P. PERRONE, JR., Assistant Examiner

U.S. Cl. X.R.

10 117-138.8 E, 138.8 F, 138.8 N, 140 A, 141, 143 A, 145,  
161 A; 260-33.8 SB, 33.8 UB